

Sept. 26, 1939.

H. L. THWAITES

2,174,021

METHOD OF AND APPARATUS FOR TESTING LUBRICATING OILS

Filed May 13, 1936

3 Sheets-Sheet 1



Fig. -1

Herman L. Thwaites Inventor

By P. P. Young Attorney

Sept. 26, 1939.

H. L. THWAITES

2,174,021

METHOD OF AND APPARATUS FOR TESTING LUBRICATING OILS

Filed May 13, 1936

3 Sheets-Sheet 2



Fig.-2

Herman L. Thwaites Inventor

By *P. H. Young* Attorney

Sept. 26, 1939.

H. L. THWAITES

2,174,021

METHOD OF AND APPARATUS FOR TESTING LUBRICATING OILS

Filed May 13, 1936

3 Sheets-Sheet 3



Fig. - 3

Herman L. Thwaites Inventor

By P. P. Young Attorney

## UNITED STATES PATENT OFFICE

2,174,021

METHOD OF AND APPARATUS FOR TEST-  
ING LUBRICATING OILSHerman L. Thwaites, Westfield, N. J., assignor to  
Standard Oil Development Company, a corpora-  
tion of Delaware

Application May 13, 1936, Serial No. 79,483

4 Claims. (Cl. 73—51)

This invention deals with an apparatus for the testing of lubricating oils, and has for its object the manufacture of a simple and inexpensive apparatus and method for determining, with reasonable accuracy, the utility of an oil for lubricating internal combustion engines.

This object is attained by the apparatus set forth in the accompanying drawings in which Figure 1 is a cross-sectional view of the cone over which the oil is passed, while Figure 2 is a diagrammatic view in partial cross-section of the cone assembly including the heating means and control mechanism. Figure 3 is a graph illustrating the correlation of results obtained with the present apparatus compared with actual engine test results.

Heretofore, in spite of the large number of lubricating oil testing apparatuses and methods, the only way in which one could determine the suitability of an oil for lubricating internal combustion engines was to actually employ such oil in such engine under controlled laboratory conditions, and examine both the used oil and the condition of the engine after the run. Such a procedure was both costly and tedious. Within recent years, a more standardized method has been developed by the use of the C. F. R. (Cooperative Fuel Research) one-cylinder engine of definite specifications and conditions of operation. This method is now considered as the most approved procedure for the evaluation of motor oils, but of course, possesses the disadvantages of high initial cost and operating expense, as well as the duration of the test. It is also subject to the additional detriment of rapid wear of moving parts requiring frequent blank runs on reference oils.

The apparatus prepared according to this invention gives results which approximate very closely the results obtained by the C. F. R. engine. Referring to the drawings, the most essential unit of the apparatus is a hollow inverted metallic cone 1 of circular cross section, having milled out in screw fashion on its inner periphery a continuous circumferential groove 2. These grooves are inclined toward the outer portion of the cone so as to facilitate circulation of the oil around the cone from the top to the bottom without interruption. The oil is allowed to flow in a continuous or discontinuous manner at the beginning of the groove at the top of the cone 2 and is slowly circulated by gravity due to the downward slope 3 of the groove to the end thereof at the bottom of the cone 4, wherefrom the

oil issues out of the cone through discharge tube 5.

This cone is preferably made of mild steel or iron, although alloy steels and other metals and alloys such as copper, aluminum, bronze, brass, and the like may be employed. It is also preferable that the test procedure be carried out in the presence of air, although other gases or vapors with or without admixture of air might be employed, such as oxygen, carbon monoxide, gasoline combustion gases, steam, carbon dioxide, formaldehyde, and the like.

In the preferred embodiment, the cone has a diameter of  $3\frac{1}{2}$ ", narrowing down over a distance of  $3\frac{3}{8}$ " to  $\frac{3}{8}$ " at the outlet tube. The wall thickness of the cone in the vicinity of the outlet tube is  $\frac{1}{2}$ ", while the height of the thread of the circular groove is  $\frac{1}{2}$ ", the depth being  $\frac{1}{4}$ ". The length of the outlet tube is  $1\frac{1}{8}$ ". The thickness of the cone wall at the top of the middle portion of the thread is  $\frac{11}{32}$ " while the thickness at the top of the cone is  $\frac{1}{8}$ ". The top of the thread surface may be rubbed down to a smooth finish with sandpaper, emery cloth, etc.

The cone 1 is mounted in a close fitting heater 6 containing resistance coils 7 capable of heating the cone to 450–550° F. This heater is mounted on tripod 8. A rheostat 9 is provided with fixed terminals 10 and 11 for supplying the required current to the heater. The temperature is maintained constant by means of adjustable slide 12, relay 13, battery 14, and mercury thermo-regulator 15. The temperature at the inner surface of the cone is measured by thermocouple 16 and potentiometer 17. A graduated dropping funnel 18, containing the oil to be tested is supported over the cone so as to slowly feed oil from the tip 19 to the first thread 2 on cone 1. If desired a cover 21 may be provided for the cone 1, which cover should be provided with openings adapted to permit the insertion into the interior of the cone of instruments 15 and 16 or the like. After the oil completes its passage over the thread it emerges through outlet tube 5 into graduate 20.

The preferred test procedure is to allow a determined volume (say 60 cc.) of the oil to be tested to flow slowly over the thread surface of the cone, allowing a time of contact of about one minute between the heated metal surface and the oil. The total volume of 60 cc. of the oil is dropped during a period of 2 hours to obtain this rate. A temperature of 250° C. (482° F.) is most desirable although lower tempera-

tures or those higher, e. g., 300° C. or even 350° C. may be used in some cases.

The cone is weighed before the test. After the fixed volume of the oil the quality of which is to be determined is run over the metal surface, the cone is washed with naphtha to remove adhering oil, dried, and the total deposit is obtained by the difference in weight. This value is generally reported in grams, the higher value showing a poorer oil. The same oil may be passed over the cone one, two, three or more times to give a better indication as to its stability upon repeated exposure on the heated cone. This may be accomplished mechanically or by the use of a recirculating pump.

The exceptionally good correlation of the results obtained by the apparatus and method disclosed herein with actual engine test results is shown in Figure 3. In the graph, the cone ratings (deposit in grams) of the various oils (denoted by the small circles) are plotted against their demerit ratings after the second 15 hour period on the C. F. R. engine. In the latter test, a definite quantity of lubricating oil is employed to lubricate a one-cylinder internal combustion engine at 390° F. jacket temperature. At the end of 15 hours, the engine parts such as the rings, grooves, piston surfaces, carbon deposits, etc., are observed, and each part is rated, the total value being the demerit rating. The same oil is then replaced in the cleaned engine which is again run for 15 hours under the same conditions, this being a more severe test since the oil has already been subjected to a previous 15 hour period. The demerit rating is then obtained on the engine parts as above, and this is the value plotted as the abscissa in Figure 3, the lower demerit rating indicating a better oil for lubrication under such conditions. In view of the poor correlation of previous chemical tests with actual engine performance, the value of the test involved in the present invention is readily apparent.

Although this test is especially applicable to viscous hydrocarbon lubricating oils, it may be likewise used to test other oils containing fatty compounds, blending agents, and the like.

An advantageous feature of the cone is its accessibility for cleaning and the ease in carrying out such operations. For instance, the thread

surface may be washed off with solvent and brush, or scraped off with emery cloth or sand-paper.

Although there have been shown and described specific embodiments of this invention, many modifications thereof are possible. The invention, therefore, is not to be restricted except insofar as is necessitated by the prior art and by the spirit of the appended claims.

I claim:

1. Apparatus for determining the quality of lubricating oil used in an internal combustion engine comprising an inverted metal cone having an inclined circumferential groove on its inner surface adapted to allow the oil to be tested to slowly flow on the top of said groove around the inner surface of the cone and through an outlet at the bottom of said cone and means for heating said cone as hereinabove set forth.

2. Apparatus for determining the quality of lubricating oils for use in an internal combustion engine, comprising a jacket having a substantially frusto-conical passageway extending along its vertical axis and a heating element disposed adjacent the walls of said passageway, an inverted metal cone, having an inclined circumferential groove on its inner surface, adapted to allow the oil to be tested to slowly flow on top of said groove around the inner surface of the cone and through an outlet at the bottom of said cone disposed in the passageway of said jacket with the outlet extending beyond the passageway, a cover for said cone, means for supplying oil to the groove and means for regulating the temperature within the cone extending through an opening in said cover.

3. Method of testing lubricating oils to determine their suitability for use in internal combustion engines, comprising passing a small stream of an oil to be tested over a confined path in a heated metal body, in the presence of a material in a substantially gaseous form, washing said metal body to remove adhering oil and weighing the residue adhering to said surface, to obtain an index of the quality of the oil.

4. A method of testing lubricating oils according to claim 3, in which the oil is maintained in contact with the heated metal body for a period of at least one minute.

HERMAN L. THWAITES.

50